

Sept. 18, 1973

T. RUMMEL

3,759,670

INITIATING THE PULLING OF A CRYSTALLINE BODY FROM A MOLTEN STOCK

Filed Sept. 18, 1970



## 1

3,759,670

INITIATING THE PULLING OF A CRYSTALLINE  
BODY FROM A MOLTEN STOCK

Theodor Rummel, Hannover-Kirchrode, Germany, assignor to Siemens Aktiengesellschaft, Berlin and Munich, Germany

Filed Sept. 18, 1970, Ser. No. 73,304

Claims priority, application Germany, Sept. 24, 1969,  
P 19 48 194.8

Int. Cl. B01j 17/18

U.S. Cl. 23—301 SP

5 Claims

## ABSTRACT OF THE DISCLOSURE

A method and apparatus for pulling a crystalline body by a seed crystal fastened in a holder from a melting stock heated, in a cold coil crucible, at least to melting temperature. The method comprises heating the holder and one end of the seed crystal, moving the preheated zone to the other end of the seed crystal, approaching the heated end to the stock to be molten, whereby the latter is heated to a temperature at which it is conductive, and thereafter, heating the stock by the field issuing from the cold coil crucible.

The invention relates to a method for pulling a crystalline body by a seed crystal fastened in a holder, from a melting stock heated, in a cold coil crucible, at least to melting temperature and to a device for performing said method.

The periodical *Laboratory Methods*, vol. LXVII, No. 404, June 1963, pages 301-307, describe a method for pulling a rod, for example silicon, from a molten liquid situated in a basket type coil crucible. This coil crucible consists of metal wire, such as for example, copper or silver, where in channels are located which are passed by a coolant, e.g. water. The outer wall of this cold coil crucible is surrounded by the winding of a primary coil. The windings are positioned in planes perpendicularly to the axis, through the crucible opening.

This primary coil is charged with high frequency AC, which induces secondary currents in the cold coil crucible. These secondary currents induce secondary currents of their own in the melting stock which is located in the coil crucible and which can thereby be heated to melting temperatures and above. One end of a second crystal, affixed at the other end within a holder, is brought into contact with the melting stock. The seed crystal is then withdrawn from the molten liquid and a monocrystalline rod, growing at the seed crystal, is pulled from the molten liquid.

The pulling of a monocrystalline body from a molten liquid located in a cold coil crucible has the advantage that the crystallized material has virtually no dislocations. Also, no undesirable impurities reach the melt liquid from the material of the cold coil crucible which is not wetted by the molten mass, and thus cannot penetrate into the crystallized rod.

If the melting stock in the cold coil crucible is a poorly conducting crystalline material, in its cold state for example, a semiconductor material such as pure silicon, this material must be preheated before it can be heated by the field, issuing from the cold coil crucible. It is known to preheat the stock by irradiating the same with a focused infrared radiation emitted by a projection lamp. During this irradiation, the primary coil which surrounds the cold coil crucible is stressed with high frequency alternating current. After the stock obtains a sufficiently high temperature, through irradiation, it is coupled to the field issuing from the cold coil crucible, and can now be further heated and melted, without the projection lamp.

## 2

However, it takes a considerable time to heat, particularly, a large amount of stock to be melted by a projection lamp, i.e. to a temperature which is high enough for the coupling process. The time required to this end is particularly protracted if the projection lamp is situated outside a recipient which contains the cold coil crucible with the crystal seed and if the radiation it emits must, for example, penetrate a quartz disc.

The invention has as its object to remedy this condition so as to heat the largest possible part of the stock to be melted, situated in the cold coil crucible by the field which issues from the coil crucible, prior to melting said stock so that the process is considerably accelerated.

The objective is achieved according to the invention, by heating the seed crystal at one end by a heating device, approaching the heated end of the seed crystal to the stock to be melted, whereby the latter may be heated and that thereupon heating the stock by the field, issuing from the cold coil crucible.

It is preferable to have the heated end of the crystal seed brought into contact with the melting stock. It is also advantageous to heat the seed crystal at one end, at least to melting temperature.

Since the crystal seed may also consist of a material which is of poor conductivity at low temperatures, a device is provided for heating the seed crystal. This device comprises an induction coil and a preheating body which may be coupled to the field of the induction coil and which is a readily conducting material.

This type of heating device may preheat the seed crystal with the aid of the preheating body, for example, at the end which is clamped into the holder. Thereafter, an incandescence zone, which is heated by the induction coil, is moved, starting at the preheated end, through a relative movement between the seed crystal and the induction coil, to the free end of the seed crystal which is then brought close to the melting stock or brought into contact with the melting stock.

The invention and its advantages will be discussed in greater detail with reference to the drawing, which shows the device.

The basket-type silver crucible 2, shown in the figure, comprises two half-rings 3a and 3b, with tubes 4a and 4b placed at their bottom, which run together at their ends. These tubes 4a and 4b are interconnected at their bottom end through a central portion 5, with channels which run together and to which tubes 4a and 4b are attached. Within the rings halves 3a and 3b are hollow spaces, within which the hollow spaces of the tubes 4a and 4b, end.

The basket-type silver crucible 2 is suspended, within a recipient, not shown in the drawing, which is either evacuated or filled with protective gas, from two hollow tubes 6 and 7. The hollow spaces of these tubes end at the hollow spaces of the ring halves 3a and 3b. Cooling water flows through tube 6, thence into the basket-type crucible 2 and leaves the same through the other tube 7, after having traversed ring half 3a, the tubes 4a, the central portion 5, the tubes 4b and the ring half 3b.

The outer wall of the basket-type crucible 2 is enclosed by a primary coil 8, which is also situated in the not-illustrated recipient and is connected to a high frequency generator, not shown.

The basket-shaped silver crucible 2, contains as the melting stock, a piece of solid, highly pure silicon 9, which attains this high electrical conductivity only at a temperature of about 600° C. so that the electromagnetic field issuing from the silver crucible 2 and induced through primary coil 8, becomes coupled to the silicon piece 9.

Above the opening of the silver crucible 2, is holder 10 on shaft 19, wherein an elongated seed crystal 11 of sili-

con is affixed. Also, above the opening of the basket-type crucible 2 is another shaft 12 at whose lower end is arranged an induction coil 13 traversed by a coolant, for example, water. The shafts 19 and 12 are displaceable in axial direction, as indicated by the double arrow. The holder 10 consists of electricity conducting steel.

Prior to the pulling process, the seed crystal 11 attached in the holder 10, is pushed through the induction coil 13 and the induction coil 13 is brought so close to the holder 10, that the coil field becomes coupled to holder 10. Thereupon, the induction coil 13 is stressed with high frequency alternating current, and the holder 10 and thus also the end of the crystal seed 11 clamped thereto, are heated to a temperature of about 600° C. Thus, a preheated zone of increased electrical conductivity develops in the seed crystal 11, in the vicinity of the holder 10. The preheated zone is coupled to the field issuing from the induction coil 13. A relative movement between the coil 13 and the seed crystal 11, causes the preheated zone of increased electrical conductivity in the seed crystal 11, to move toward the end of the seed crystal. The induction coil 13 is so strongly stressed with energy that the lower end of the seed crystal 11 melts. The coil 13 and the seed crystal 11 are now moved so far downward until the molten drop contacts the to be molten stock 9, consisting of cold silicon. As a result, a region of several cubic centimeters is heated in the stock 9, to a temperature of at least 600° C. In this range, the field issuing from the basket-type silver crucible 2, becomes coupled, so that gradually, the entire stock 9 is molten through the energy, supplied to primary coil 8, and is heated thereby. Thereupon, the current supply to the induction coil 13 is interrupted and the induction coil 13 is shifted axially to the holder 10. Subsequently, the holder 10 is removed together with the coil 13, axially upward, and a rod-shaped crystal growing at the lower end of the seed crystal 11, is pulled from the molten silicon, in the basket-shaped silver crucible 2.

Under certain circumstances, it is sufficient to heat the lower end of the seed crystal 11, only to glowing temperature. Also, the energy supply to the induction coil 13 may be disconnected immediately after the crystal seed 11 and the solid molten stock 9, are brought into contact. Finally, a separate preheating device which may be coupled to the induction coil 13, may be located beneath the holder 10, such as a molybdenum ring across which the induction coil 13 may be so pushed that the ring will not cause interturn short circuit.

The silicon, in the silver crucible 2, may weigh several hundred grams while the monocrystalline silicon seed crystal 11 has a diameter of 4 mm. The power of the induction coil 13 is, in this case, about 2 kw. The frequency of the high frequency AC current, with which the primary coil 8 is charged, is within the range of 0.5 to 1 mHz., while the output of the coil 8 is about 60 kw.

Although the crucible 2 is specifically described as being silver, it can also be copper, as previously mentioned.

What is claimed is:

1. A method for pulling a crystalline body by a seed crystal fastened in a holder from a melting stock heated, in a cooled, multiwinding induction heating coil crucible, at least to melting temperature, which comprises heating inductively, said holder and adjacent end of the seed crystal by an inductive heating device, utilizing said holder

to facilitate developing a preheated zone of increased electrical conductivity in said heated end of said seed crystal, providing relative movement between said inductive heating device and said seed crystal, moving said preheated zone of increased electrical conductivity toward the other end of said seed crystal, approaching the heated end to the stock to be molten, whereby heat from the seed crystal heats the stock to a temperature at which said stock is conductive, and thereafter heating said stock by the field issuing from the cooled multiwinding coil crucible.

2. The method of claim 1, wherein the heated end of the seed crystal is brought in contact with the stock to be melted.

3. The method of claim 1, wherein the one end of the seed crystal is heated at least to melting temperature.

4. The method of claim 1, wherein an induction coil and a preheating body which may be coupled to the field of the induction coil and is a readily conducting material are provided for heating the seed crystal.

5. Apparatus for pulling a crystalline body from a melting stock which comprises a cooled, multiwinding induction heating coil crucible, an induction coil surrounding said crucible, a seed crystal holder above the opening of said crucible, a seed crystal in said seed crystal holder, a movable induction coil surrounding said seed crystal and initially disposed about the end of said seed crystal adjacent to said holder whereby said moveable induction coil heats said holder and a preheated zone of increased electrical conductivity is developed in the end of said seed crystal adjacent to said holder, said moveable induction coil being moveable relative to said seed crystal so that said preheated zone of increased electrical conductivity is first moved to the other end of said seed crystal to melt said other end of said seed crystal and means to subsequently approach the said other end of the seed crystal with the stock in the crucible to be molten.

#### References Cited

##### UNITED STATES PATENTS

|           |         |               |       |        |
|-----------|---------|---------------|-------|--------|
| 2,664,496 | 12/1953 | Brace         | ----- | 23—301 |
| 2,793,103 | 5/1957  | Emeis         | ----- | 23—301 |
| 3,069,244 | 12/1962 | Sterling      | ----- | 23—301 |
| 3,086,850 | 4/1963  | Marino et al. | ----- | 23—301 |
| 3,090,673 | 5/1963  | Sterling      | ----- | 23—301 |
| 3,172,734 | 3/1965  | Warren        | ----- | 23—301 |
| 3,258,314 | 6/1966  | Redmond       | ----- | 23—301 |
| 3,494,804 | 2/1970  | Hanks et al.  | ----- | 23—301 |
| 3,505,025 | 4/1970  | Dessauer      | ----- | 23—273 |

##### FOREIGN PATENTS

|           |         |           |       |        |
|-----------|---------|-----------|-------|--------|
| 230,742   | 10/1960 | Australia | ----- | 23—273 |
| 233,354   | 4/1961  | Australia | ----- | 23—301 |
| 1,108,543 | 4/1960  | France    | ----- | 23—301 |
| 1,289,950 | 2/1969  | Germany   | ----- | 23—301 |
| 1,326,841 | 4/1963  | France    | ----- | 23—301 |

NORMAN YUDKOFF, Primary Examiner

R. T. FOSTER, Assistant Examiner

U.S. CL. X.R.

23—273 SP; 219—10.43